

## UNITED STATES PATENT OFFICE.

FRANCIS GRIMSHAW MARTIN, OF HIGHER BEBINGTON, ENGLAND.

## MANUFACTURE OF MILD-STEEL PLATES, SECTIONS, AND THE LIKE.

No Drawing. Application filed February 17, 1925, Serial No. 9,880, and in Great Britain January 26, 1925.

This invention has reference to the manufacture or production of mild steel plates, sections, or the like, in which the unequal elastic limit of the plate, section, or material, in both the longitudinal and lateral or different directions, produced by the usual rolling or forging is removed, and also the deformed structure of the said steel is restored.

10 In a prior patent application Serial No. 630,389, of which the present applicant, F. G. Martin, is the applicant, a process is described of producing mild steel plates or material for use in ship building, in which 15 these effects or results are accomplished; and it is found that, by the adoption of that process or treatment, not only are the said effects produced in the plates or material, but also their elastic limit test is much higher 20 than in ordinary mild steel plate or material, in the ratio of at least about 15 to 8. That is, the elastic limit of the original mild steel has been raised by the process or treatment in the ratio of at least 8 to 15, 25 with the result that ships of mild steel can be built of very substantially less weight than heretofore, as therein stated.

The present application for patent is for the manufacture and use of mild steel plates, 30 sections, or the like, for structures other than ships—such as bridges, and other plate and girder work, buildings, vehicles, boilers, rolling stock, and the like, in which the work is subjected to more or less severe 35 stresses—produced by the process or treatment, consisting of heating them throughout to 800° to 900° C., and subsequently rapidly cooling them by causing currents of air to pass over their surfaces, or where 40 suitable or convenient by immersing them in or subjecting them to water or oil.

This heat treatment or process produces plates or material having the characteristics stated, and enables relatively thin plates or 45 material to be safely used in structures such as referred to, which are subjected to large or substantial stresses.

All the material proposed to be used in the structure should be tested both for their 50 longitudinal elastic characteristics, and their transverse elastic characteristics; and

this may be effected by testing edge trimmings cut from the side edges or margins of the heat treated plates, material, or members, and those taken from their end edges or margins, so that it will be ascertained whether the elastic qualities required in the plate in the different directions, are equal, and of the standard required.

To enable these testings to be quickly 60 performed, test pieces of T-headed form may be cut out of the said longitudinal and lateral trimmings or margins in any suitable way, and their heads are placed in a testing machine having grippers of a kind 65 which enable them to be quickly put in, gripped, tested, and taken out.

Such a mechanism is illustrated in the specification of the said former application for patent, Serial No. 630,389, and de- 70 scribed therein.

By this means rapid and accurate testing of a large proportion of, or every plate and section or member of mild steel used can be effected, and the elastic limit of every tested 75 plate, section or member used known, so that it is not necessary to assume large factors of safety in plates, sections, or material used in bridge work, girder work, boilers, and other structures, subject to stress, 80 as has been hitherto deemed to be necessary; and by this invention relatively thin plates can be safely used resulting in a relatively light structure.

## What is claimed is:—

A process for treating mild steel plates which through their rolling or forging treatment have produced a steel with a material inequality of longitudinal and lateral elastic limits, consisting in heating the 90 plates to between 800° and 900° centigrade and then rapidly cooling the plates artificially to thereby equalize the elastic limit in all directions, and materially increase such elastic limit over that of the plates as 95 rolled or forged without in any particular increasing the hardness of the steel as a result of the process.

In testimony whereof I have signed my name to this specification.

F. G. MARTIN.